

## UNITED STATES PATENT OFFICE

1,989,643

PNEUMATIC INNER TUBE AND METHOD OF  
MAKING ITPaul W. Litchfield, Akron, Ohio, assignor to Wing-  
foot Corporation, Wilmington, Del., a corpora-  
tion of DelawareNo Drawing. Application March 17, 1931,  
Serial No. 523,384

12 Claims. (Cl. 18—56)

This invention relates to pneumatic inner tubes for vehicle tires that are to be substantially stretched during use. It includes the new tubes and the method of making them. More particularly, the invention relates to inner tubes having a coating film upon the surface which will prevent or retard the loss of inflating gas by diffusion through the walls.

It has heretofore been observed that where inner tubes for pneumatic tires are left inflated for a considerable period of time, the inflating medium (usually air) tends to diffuse through the walls of the tubes and escape to the outer atmosphere, thus permitting a gradual loss of pressure within. Since it is highly desirable to maintain a uniform pressure within inner tubes in order to insure the degree of inflation requisite to obtaining maximum durability in the enclosing casing, such loss of inflating gas is highly undesirable.

This invention comprises the provision of a coating medium which, when applied to the surface of an inner tube, effectively prevents the diffusion of the inflating gas through the walls of the tube, thereby insuring proper inflation at all times. Various media may be employed for coating the tubes. However, in most cases, best results are obtained by employing a medium containing an appreciable proportion of gelatin, glue or other similar gel-forming hydrophylic colloid material.

Excellent results may be obtained by the use of a film comprising a latex of the type from which rubber, balata or gutta percha is obtained, together with gelatin and a plasticizing agent, such as polyglycerol or the like. With this coating, best results are obtained by employing a plurality of thin films upon the surfaces to be coated. The inner of these films should contain a relatively large proportion of latex while the proportion of latex is gradually decreased in the outer coatings and, in lieu thereof, gradually increasing proportions of gelatin or similar material are substituted. The following is a specific example of a formula involving a number of cements which, when employed in the order indicated, has been found by actual test to yield excellent results. The cement is applied directly to the tube, then the composition containing no

gelatin or polyglycerol and then the other compositions in the order listed.

| Solution:                      | Cone.<br>latex<br>58%<br>solids | NaOH | Gel-<br>time | Poly-<br>glycerol | H <sub>2</sub> O | Wt. of<br>solution<br>g. per sq.<br>in. | 5  |
|--------------------------------|---------------------------------|------|--------------|-------------------|------------------|-----------------------------------------|----|
| Cement<br>(ordinary<br>rubber) |                                 |      |              |                   |                  |                                         | 44 |
| #1                             | 48.2%                           | 1.8% |              |                   |                  | 50.5%                                   | 33 |
| 2                              | 19.3                            | 0.5  | 54.4%        | 10.8%             | 64.0             | 61                                      | 10 |
| 3                              | 6.9                             | 0.2  | 7.7          | 15.4              | 69.8             | 110                                     |    |
| 4                              |                                 |      | 9.0          | 18.0              | 73.0             | 121                                     |    |
| 5                              | 6.9                             | 0.2  | 7.7          | 15.4              | 69.8             | 144                                     |    |
| #2                             | 19.3                            | 0.5  | 5.4          | 10.8              | 64.0             | 121                                     | 15 |

(The polyglycerol referred to in this table was obtained by heating glycerine to a temperature of about 300° C. in the presence of a small amount of some catalyst such as caustic soda or iodine.)

In applying these various films to an inner tube for pneumatic tires, it is preferable to dispose the tube containing the usual compounding ingredients in the green or uncured state upon a mandrel of proper diameter which may be either straight or curved. The films may then be applied by brushing, spraying or dipping, each film being permitted partially to dry before application of the succeeding one. After application of the films, the tubes are permitted to stand for a sufficient period of time to allow substantially complete evaporation of the volatile liquids contained within the coating materials. The tubes may then be stripped from the mandrels and turned inside out to dispose the coated surface within the interior thereof. The ends are then joined to form an annulus, after which the whole is subjected to vulcanization within molds in the ordinary manner.

It is also possible to cure the tubes directly upon the mandrels and then to strip them and turn the coated surface inwardly by the same method employed in stripping the uncured tubes. The ends of the cured tubes may then be buffered, cemented and spliced in the same manner as the ordinary mandrel cured tube. In this latter method of manufacture, it is, of course, to be understood that a medium which will not absorb the gelatin and polyglycerol from the coating film should be employed in the heaters in

5

10

15

20

25

30

35

40

45

50

which the tubes are cured. Heated gas, such as nitrogen or carbon dioxide, produces most satisfactory results for this purpose.

The coating films, when thus applied to the inner tubes, adheres so firmly to the surface of the tubes that they appear to be blended with the rubber constituting the main body of the tube and for that reason, the tubes may be stretched and flexed without any tendency to cause separation between the film and the rubber upon which the latter is disposed. Also, in spite of repeated stretching and flexing, the continuity of the film is not broken. Therefore, the impermeability of the film to inflating media, such as air or other gases, is unimpaired.

The efficiency of the coating medium as a means of preventing diffusion of inflating fluid from within a tube of the size employed in a tire having a cross-sectional diameter of 4.75 inches and a bead diameter of 19 inches was determined by inflating the tube when enclosed within a standard tire casing to a pressure of 35 pounds per square inch. The tube was left standing for a period 24 days, after which the pressure therewithin was determined. The loss was found to be approximately one pound per square inch. The tire containing the tube was next placed upon the revolving shaft of a resiliometer and run in contact with a drum having cleats disposed upon the surface thereof until the outer periphery of the tire had traveled a linear distance of 2000 miles. The pressure test was then repeated. It was found at the conclusion of the test that there had been no appreciable loss during the latter period. Even this slight loss was probably accounted for by reason of the escape of air through the valve of the tube when the gauge was applied for purposes of determining the pressure.

In a similar tire containing an inner tube identical in construction except for the omission of the coating films, the pressure drop at the end of the 24 day period amounted to 14 pounds per square inch and, at the end of the test upon the resiliometer, the total drop was 15½ pounds per square inch.

In the above described coating media, as has already been indicated, the gelatin appears to constitute the principal gas-stopping agent. For that reason, the latex may be entirely dispensed with or it may be replaced by artificial suspension of rubber, such as the ordinary cement of rubber and gasoline or rubber and benzene. However, it is always desirable to retain a suitable plasticizing agent, such as polyglycerol, Turkey red oil, or similar material in the gelatin film. While in the previously described films, gelatin constituted the principal agent, it is understood that materials having similar properties may, in some cases, be substituted therefor with fairly satisfactory results. For example, glue, casein, haemoglobin or other gel-forming hydrophylic colloids of similar character may, if properly plasticized by polyglycerol or similar agent, be employed. Where these substances are employed as coating media, it is highly desirable that the pressure fluid contacting with the coated surface during cure or subsequent use of the articles be substantially free from water and water vapor in order to prevent undue softening of the coating agent. The material should also be free from tanning agents, which may cause peeling of coating from the surface to be protected.

The new coating medium is inexpensive to

prepare and may be applied to the surfaces of the inner tubes with great ease. In view of the high efficiency thereof as means for preventing the escape of inflating gas, its use is highly desirable from a commercial viewpoint.

5

Although I have disclosed only the preferred forms of the invention and have described those forms in detail, it will be apparent to those skilled in the art that the invention is not so limited but that various modifications may be made therein without departing from the spirit of the invention or from the scope of the appended claims.

10

What I claim is:

1. A pneumatic rubber inner tube for vehicle tires having a coating upon at least one surface thereof, said coating being substantially coextensive with said surface and comprising a composition containing gelatin and a polyglycerol.

2. A pneumatic rubber inner tube for vehicle tires having a coating upon at least one surface thereof, said coating being substantially coextensive with said surface and comprising a composition containing latex, gelatin and a plasticizing agent.

25

3. A pneumatic rubber inner tube for vehicle tires having a coating upon at least one surface thereof, said coating being substantially coextensive with said surface and comprising a composition containing latex, gelatin and a plasticizing agent, said coating further comprising a plurality of films, the proportion of latex being gradually decreased and the proportion of gelatin gradually increased in each film from the inner to the outer film.

30

4. A pneumatic rubber inner tube for vehicle tires that is to be substantially stretched during use said tube being coated with an extensible gas impervious film capable of adhering closely and stretching with the tube without rupturing or separating from the tube.

35

5. A pneumatic rubber inner tube for vehicle tires that is to be substantially stretched during use said tube being coated with an extensible gas impervious film capable of adhering closely and stretching with the tube without rupturing or separating from the tube, said coating containing a gel-forming hydrophylic colloid and a plasticizer.

40

6. A pneumatic rubber inner tube for vehicle tires that is to be substantially stretched during use said tube being coated with an extensible gas impervious film capable of adhering closely and stretching with the tube without rupturing or separating from the tube, said coating containing a gel-forming hydrophylic colloid, rubber and a polyglycerol.

45

7. A pneumatic rubber inner tube for vehicle tires capable of withstanding repeated stretching and flexing and coated on at least one surface with a dried gas impervious film which will stretch and flex with the tube without rupturing or separating therefrom, said coating containing a gel-forming colloid and polyglycerol.

50

8. A pneumatic rubber inner tube for vehicle tires that is to be repeatedly stretched and flexed in use, which includes an extensible gas impervious film adhered to at least one surface thereof, said film having been applied prior to the vulcanization of the rubber and being capable of retaining its adhesion to the tube throughout repeated stretching and flexing.

55

9. The method of making a pneumatic rubber inner tube for vehicle tires which comprises dis-

70

75

posing the tube containing the usual compounding ingredients in an uncured state upon a mandrel, applying to the exposed surface of the tube a gelatin-containing film in a vehicle, then after 5 substantially complete evaporation of the vehicle stripping the coated tube from the mandrel, turning it inside out, joining the ends and then subjecting the whole to vulcanization.

10. The method of making a pneumatic rubber inner tube for vehicle tires which comprises disposing the tube containing the usual compounding ingredients in an uncured state upon a mandrel, applying to the exposed surface of the tube a gelatin-and-polyglycerol-containing film 10 in a vehicle, then after substantially complete evaporation of the vehicle stripping the coated tube from the mandrel, turning it inside out, joining the ends and then subjecting the whole to vulcanization.

15 20 11. The method of making a pneumatic rub-

ber inner tube for vehicle tires which comprises disposing the tube containing the usual compounding ingredients in an uncured state upon a mandrel, applying to the exposed surface of the tube a gel-forming hydrophyllic colloid and a plasticizer, stripping the coated tube from the mandrel, turning it inside out, joining the ends and then subjecting the whole to vulcanization.

12. The method of making a pneumatic rubber inner tube for vehicle tires which comprises disposing the tube containing the usual compounding ingredients in an uncured state upon a mandrel, applying to the exposed surface of the tube a gelatin-latex-polyglycerol-containing film in a vehicle, then after substantially complete evaporation of the vehicle stripping the coated tube from the mandrel, turning it inside out, joining the ends and then subjecting the whole to vulcanization.

PAUL W. LITCHFIELD. 20